

# United States Patent Office.

LEOPOLD BRANDEIS, OF BROOKLYN, NEW YORK.

*Letters Patent No. 70,513, dated November 5, 1867.*

## IMPROVED ALLOY FOR THE MANUFACTURE OF METAL SHEETS, FOIL, &c.

The Schedule referred to in these Letters Patent and making part of the same.

### TO ALL WHOM IT MAY CONCERN:

Be it known that I, LEOPOLD BRANDEIS, of the city of Brooklyn, county of Kings, and State of New York, have invented a new and useful Process for the Manufacture of a New and Superior Roofing Material, suitable at the same time for plumbers' use, for chemical works, and for making canisters, capsules, caps for bottles, and for packing dry substances like tea, coffee, spices, tobacco, chocolate, &c.

I will proceed now to describe my process, which is divided into two parts: the first part including the material used for roofing and other purposes where strength, pliability, and resistance to the changes of temperature and weather are required; the second, where a thin and still stiff covering is wanted to exclude moisture and avoid thereby mouldiness or fermentation.

To produce the article for roofing and other purposes mentioned, I prepare an alloy of twenty-five per cent. zinc, seventy-five per cent. of lead. This alloy has all the advantages of pure lead, while it is cheaper, tougher, and more durable. This alloy I coat with tin, or surround the ingots with cylinders of tin and roll it out. I can cast these ingots in any suitable shape, or press them out of a die by means of hydraulic pressure. By means of chilled-iron or steel rollers I produce sheets from two pounds to ten pounds per square foot. These sheets, properly folded and pressed down, do not require any soldering on the roof, but the outside being a solid covering or coat of tin, will resist oxidization far better than any metallic substance used so far, will be less liable to contraction and expansion than sheet iron tinned, (tin plate,) and will answer better than sheet lead for cisterns, plumbers' work, chemical works, &c., &c.

The second part of my process consists in preparing thinner sheets of the tinned alloy for lining boxes, and for making thin sheets used for wrapping purposes. I make for this purpose an alloy containing, according to the special use of the article to be manufactured, between ten and fifteen per cent. zinc, and ninety per cent. to eighty-five per cent. of lead. I coat this also with tin, after casting or pressing suitable ingots of any desirable shape or size. But to enable me to roll it as thin as may be required, I expose the metal to the action of hot water, (at 212°.) or to steam between the rollings that may be required to bring it to its proper degree of thickness, so as to keep the metal perfectly ductile during this operation. My sheets, by the mixture of zinc and lead, get stiffer and stronger without losing their pliability, or without increase of weight.

I do not claim to produce tin-foil by covering lead, either hot or cold, with tin, and by rolling these metals out together; nor do I claim to make a covering or cylinder of tin first, and to fill this with hot or cold lead by casting, hydraulic or other pressure, as this has been done before; but

I claim to produce metal sheets of any thickness, perfectly pliable, not easily acted upon by weather and temperature, of great strength and durability for roofing, plumbers', tinmen's, and chemical use, for grocers, tobacconists, perfumers, and confectioners, by making an alloy of lead and other metals in suitable proportions and shape, by protecting this alloy with a coat of tin surrounding it, and to produce from this alloy, so prepared, sheets or leaves of any size and weight, and for the device of application of hot water or steam between the rollings.

LEOPOLD BRANDEIS.

Witnesses:

HERMAN WISCHMANN,  
WM. KELLOGG.